

## UNITED STATES PATENT OFFICE

1,996,120

MANUFACTURE OF ARTIFICIAL THREADS  
OR FILAMENTS

Reginald William Payne and Robert Pierce  
Roberts, Spondon, near Derby, England, as-  
signors to Celanese Corporation of America, a  
corporation of Delaware

No Drawing. Application December 12, 1928,  
Serial No. 325,479. In Great Britain December  
23, 1927

2 Claims. (Cl. 18—54)

This invention relates to the manufacture of  
artificial filaments or threads from solutions of  
cellulose acetate or other esters or ethers of cellulose  
by the dry spinning or evaporative method  
of formation.

In the spinning of such artificial threads or  
filaments by the dry or evaporative method of  
formation, solutions of organic cellulose derivatives  
(that is cellulose acetate or other esters or  
ethers of cellulose) in volatile solvents are spun  
into an evaporative atmosphere (usually into a  
current of heated air) the threads or filaments  
so formed being continuously wound up, with  
or without twisting, on apparatus situated within  
or outside the evaporative atmosphere. The  
threads or filaments heretofore produced by such  
method of spinning have been lustrous in char-  
acter and have found successful application as  
artificial silk, artificial horse hair and the like.

The object of the present invention is to pro-  
duce threads or filaments presenting reduced  
lustre and more particularly threads or filaments  
presenting a dull matt or lustreless appearance,  
or of considerably reduced lustre.

For this purpose, according to the invention, we  
employ solutions of cellulose acetate or other  
organic esters or ethers of cellulose in volatile  
solvents and containing water, and we perform  
the spinning of said solutions by the dry or  
evaporative method under such conditions that  
the water exerts a precipitating action on the  
filaments in the natal state of the filaments.

In performing the invention we may extrude  
into a heated casing or spinning cell (such for in-  
stance as described in U. S. Patents Nos. 1,602,125  
and 1,541,104 and 1,731,317), through which a  
current of air is caused to pass, a solution con-  
taining cellulose acetate or other esters or ethers  
of cellulose and water. The quantity of water  
present in the spinning solution will vary accord-  
ing to the spinning conditions and the result it is  
desired to achieve.

In general, quantities of water from about 10%  
or less to 30% or more, and preferably 20% to  
30%, relatively to the volatile solvent should be  
employed, but it will be understood that these  
quantities are only given by way of illustration.

The quantity of water employed in the spinning  
solution should of course be sufficient to cause a  
precipitation of the cellulose derivatives from  
solution under the spinning conditions employed.

The following example serves to illustrate one  
form of the invention.

## Example

Highly satisfactory filaments, threads or yarns  
presenting reduced lustre may be produced by  
extruding any of the following solutions into an  
evaporative atmosphere of heated air, for in-  
stance, downwards into a heated metier casing or

spinning cell through which a current of air is  
caused to pass in an upward or downward direc-  
tion.

## Solution

[Parts by weight]

|                           | <i>a</i> | <i>b</i> | <i>c</i> | <i>d</i> | <i>e</i> | 5  |
|---------------------------|----------|----------|----------|----------|----------|----|
| Acetone 99-100% pure..... | 72       | 76       | 78       | 84       | 92       | 10 |
| Water.....                | 28       | 24       | 22       | 16       | 8        |    |
| Cellulose acetate.....    | 33½      | 33½      | 33½      | 33½      | 33½      |    |

The degree of delustration produced will vary  
with the temperature of the heated air. Thus  
with a current of air heated to a temperature of 15  
50° C. each of the above solutions will yield de-  
lustrated artificial filaments, the filaments pro-  
duced from solutions *a* or *b* being substantially  
completely delustrated and presenting a dull matt  
appearance, the filaments produced from solu-  
tions *c* or *d* being very dull but slightly more  
lustrous than those produced from solution *a* or  
*b*, whereas filaments produced from solution *e*  
are only slightly delustrated. With increasing  
temperatures of the heated air the degree of 25  
delustration imparted to the filaments will de-  
crease, for instance, with a current of air heated  
to a temperature of 65° C. solutions *a* or *b* yield  
slightly delustrated filaments, whereas solutions  
*c* or *d* yield bright filaments of but slightly re-  
duced lustre. Solution *e* should not be spun with  
an air current exceeding temperatures of about  
50° to 60° C., otherwise the water will not act as a  
precipitant and highly lustrous filaments will  
result. 35

In performing the invention we preferably wind  
the filaments up (continuously with their forma-  
tion) with or without twisting, on apparatus lo-  
cated outside the evaporative atmosphere, though  
such winding may be performed within said at-  
mosphere if so desired. 40

It is to be understood that the invention is in  
no way limited to the particular example of ex-  
ecution described which may be varied widely.

The filaments may be extruded either down-  
wards or upwards into the spinning cell or metier  
casing, and the air current (which may be caused  
to pass either upwards or downwards through  
the metier casing or cell) may be heated or  
warmed therein or prior to admission thereto or  
both before and during passage through the cell  
or metier casing. Further, the filaments may be  
extruded in the same direction as or counter-cur-  
rent to the air current. 50

The temperature to be employed in the spin-  
ning cells or metier casings may vary with the  
boiling point of the solvents used, the composition  
of the spinning solutions and the degree of delus-  
tration it is desired to produce in the filaments or  
threads. Such temperatures may be higher or 55  
60

lower than the boiling point or points of the solvent or solvents employed.

We have found that with spinning solutions containing the more usual solvents such as acetone, methyl acetate or the like, temperatures of about 40° to 80° C. may usefully be employed in the spinning cells or metier casings, but we in no way limit ourselves to such temperatures.

By means of the present invention it is possible to obtain threads or filaments showing any desired degree of reduced lustre, from a completely delustrated or matt appearance to a relatively high lustre according to the proportion of water present and the spinning conditions employed. In general, the greater the proportion of water present in the spinning solution the greater will be the degree of delustration obtained under similar spinning conditions, and the greater the temperature employed for spinning a solution of given water content the less will be the degree of delustration obtained.

What we claim and desire to secure by Letters Patent is:—

1. Process for the production of artificial filaments presenting reduced luster comprising forming filaments from solutions of cellulose acetate in a volatile solvent comprising acetone and between 10% and 30% of water, relatively to the volatile solvent, by the dry or evaporative method under such conditions that the water exerts a precipitating action on the filaments in the natal state of the filaments. 5

2. Method of producing artificial filaments presenting reduced luster which comprises extruding into a current of air heated to a temperature between 50° and 65° C. a solution of cellulose acetate composed of between 72 and 84 parts of acetone, between 28 and 16 parts of water and 33½ parts of cellulose acetate. 15

REGINALD WILLIAM PAYNE. 20  
ROBERT PIERCE ROBERTS.